

## UNITED STATES PATENT OFFICE

ABRAHAM JOFFÉ, OF LENINGRAD, UNION OF SOCIALIST SOVIET REPUBLICS, ASSIGNOR  
TO INDUSTRIAL RESEARCH COMPANY, OF CAMBRIDGE, MASSACHUSETTS, A COR-  
PORATION OF MASSACHUSETTS

PROCESS FOR FORMING ON THE SURFACE OF A DIELECTRIC A THIN LAYER, IN  
WHICH THE POTENTIAL FALL IS CONCENTRATED

No Drawing. Application filed January 12, 1927, Serial No. 160,772, and in Germany August 3, 1926.  
Renewed June 1, 1929.

My invention relates to insulators and dielectrics and aims to make them resistant to extreme potentials. An object of my invention is to accomplish the above with a minimum of insulating or dielectric material.

5 My new and improved insulator or dielectric can withstand such extreme potentials for such a little thickness of material, that enormous quantities of energy may be stored therein. Thus, if used as a dielectric in an electric condenser, the energy stored in the condenser as a whole, which is a function of the potential applied and the capacity of the condenser, may be many times what is now 10 possible for the same size. Furthermore, if in a condenser, the plates are allowed to come close together or separate, the attractive forces due to a variation of the electrostatic field, will vibrate the plates in accordance with the 15 fluctuation of the field. This phenomenon is well known and has been taken advantage of to design electrostatic voltmeters, telephone receivers, etc. My new and improved dielectric, by greatly increasing the potentials that 20 may be used, and increasing the capacity of the condensers, allows the generation of enormous attractive and repulsive forces in this manner.

25 A further desirable result secured by my invention is the possibility of having comparatively little and cheap insulation do the work—and in a better way—of the very complicated and highly expensive insulation now used in cables for high voltage transmission of electricity. The very wasteful and 30 extremely undesirable silent discharge is entirely eliminated.

35 Inasmuch as the design and manufacture of my improved insulation and dielectric, though extremely simple, depends in a great measure upon a proper appreciation of the theory upon which it works, I shall first state what I consider to be the drawbacks and causes of failure of present day insulation. 40 Then I shall state my theory for such failure and disclose my new and improved insulation and methods of making it. Although I have based much of my work upon the lines delineated by my theory and have obtained results in accord with the same theory, yet it is

only a theory, subject to future changes and possible rejection, and therefore, I do not wish to be bound by it. I merely offer it as an aid to a proper understanding of my invention. What I offer as a disclosure in return for the 45 patent protection desired is the results obtained thereunder.

50 My researches in the field of insulators and dielectrics convinced me that the real underlying cause of their breakdown is the generation of many ions by impact with the consequent conduction of an electric current therethrough. Thus we will consider a conductor with a coat of ordinary insulation. It is well known that there exist a number of 55 free ions in the air and in most substances under ordinary conditions. How they are generated is not generally known. The sun with its radiant energy of various wave lengths, X rays, and radio-active substances 60 in the earth, and other similar causes, is undoubtedly responsible for the existence of many of these free ions. The number is variable and depends upon such factors as 65 time of day, season, weather, etc. If such a 70 free ion happens to wander into an electric field, such as might be produced by the potential which is impressed on our conductor, this ion will be drawn so that it tends to approach an oppositely charged pole. Thus, 75 80 if the ion is a positively charged one, and the conductor is charged positively, the ion will be repelled from it and drawn toward the negatively charged pole which may be either another conductor or ground. As is 85 well known, a charged particle which is in a potential field, starts from a position of 90 rest, at which position, its potential energy is a maximum and kinetic energy is a minimum, and is gradually accelerated toward the opposite pole. When this particle has fallen through the entire potential, its potential energy is now zero, while its kinetic energy 95 is a maximum. In the case at hand, however, such a particle could hardly fall through the entire potential uninterruptedly. In our case there will undoubtedly be some free ions in the insulation material adjacent the conductor. Many of these, due to the polarity of 100 the conductor will be repelled from it. Such

a particle will have its acceleration always perpendicular to equipotential surfaces. As may be understood, the steeper the potential gradient, the greater the acceleration on the particle. Such a particle will, therefore, be travelling at a high speed in a comparatively short distance. The course of this particle under ordinary conditions is beset with the molecules composing the substance or medium in which it happens to be; here the medium would be the insulation. The result is that this accelerated ions, instead of pursuing a straight and direct course, probably pursues a very tortuous course, bumping into molecules, rebounding, getting up speed again, bumping again and so on. Above a certain critical potential gradient, called the ionizing potential gradient, such an ion would be accelerated sufficiently within a distance of between 1 and 5 microns, so that if it collided with a molecule, the force would be sufficient to break up the molecule into separate and oppositely charged ions. Each of these ions would, of course, be attracted towards the pole having an unlike charge. Furthermore such ions would act the same way as the original free ion and would create other ions.

This state of affairs may be shown by a very simple equation. If  $D$  is the actual thickness of the insulator on our conductor, and if  $X$  is the distance within which the ion gets up sufficient speed to cause an ionizing impact with a molecule, then  $Z$ , the number of collisions of one originally free ion, will be equal to

$$\frac{D}{X}$$

after which collision, the number of free or detached ions present is doubled. It is readily apparent, therefore, that the number of ions increases exponentially. Thus the number of ions,  $N$ , formed from one original ion, equals  $2$  raised to the  $Z$ th power, where  $Z$  is the number of collisions as above.

$$N=2^Z$$

As was stated above,  $X$  is a very small number as a rule, and since  $D$  is usually very much greater than  $X$ ,  $Z$  will be very large, while  $N$  will be enormous. To take a concrete case, imagine that the insulation on our conductor is about one quarter of an inch thick. This corresponds to about  $6\frac{1}{3}$  mm. Assuming 5 microns or  $.005$  mm. as  $X$ , which is a probable maximum under ordinary conditions, then  $Z$  would come out about 1300.  $N$  would therefore, be equal to  $2$  raised to the 1300th power. This number is almost inconceivable, there being between four and five hundred figures. Our ordinary numbers, even to billions, form but a very small fraction of such a number. When it is considered that this number of ions is formed by only one free ion

in the first place, it will be readily apparent that the grand total will be still greater when multiplied by the number of free ions. Such a flow of ions is equivalent to a heavy flow of current, and as a matter of fact, a short circuit occurs when such a state of affairs is reached.

With present types of insulation, the potential gradient must be kept below the ionizing gradient to avoid the above effects. This imposes a maximum stress on such insulation beyond which it is impossible to go, if the insulation is to last any length of time. Since the gradient is merely the fall of potential through a unit distance, it can readily be seen that if very great potentials are to be insulated properly, the thickness of insulation must be greatly increased in order that the potential gradient remain below the ionizing point. In my new and improved insulation, the entire fall of potential is taken up by a very thin polarized layer. I have experimentally proven that the gradient or drop of potential per unit distance was the same at all parts of the polarized layer. The gradient, therefore, depends upon the thickness of this layer. Between the limits of a little less than 1 micron and about 5 microns of thickness, the potential that can be safely insulated by this layer, is practically independent of the thickness of the layer. This latter fact is not true of present day insulation.

It is to be distinctly understood that it is only the polarized layer that really performs the function of an insulator. If such a layer be formed on glass or mica, which is not polarized, has very little potential drop across it, and may be considered as a means of support for the polarized layer. Hence such support may be as thick or as thin as desired. It is possible to have this layer on each side of the insulator or dielectric, or a series of these layers may be obtained by superposing laminations of insulating material, each one having polarized layers thereon. In such a case it is essential that no continuous ionic path be provided whereby substantial impact ionization might occur. A composite insulator of this kind may be produced by having several laminae of linseed oil varnish, each lamina treated to obtain a polarized layer. It seems that the linseed oil varnish proper is sufficiently conducting so that any ions that come to it are conducted away and thus no very great amount of cumulative ionization is possible on the other side of the linseed oil varnish proper is sufficiently conducting so that any ions that come to it are conducted away and thus no very great amount of cumulative ionization is possible on the other side of the linseed oil varnish. With a linseed oil laminated insulator, each lamina treated to obtain a polarized layer, and the entire insulator being but 200 microns thick, I have

impressed 60,000 volts across it without causing a breakdown. Such a potential corresponds to  $3 \times 10$  to the 6th power volts per cm., whereas the maximum potential gradient for ordinary insulation is about  $2 \times 10$  to the 5th volts per cm., and at that potential gradient it is dangerously close to the ionizing point.

Using the above insulator in a condenser 10 through which high frequency current was passed, the condenser conducted 10 amperes at 10,000 volts. The loss angle of the insulator under these conditions was only  $2^\circ$ . As is well known, an ideal dielectric has no 15 loss angle at all, and in an ideal condenser, the current leads the potential by exactly  $90^\circ$ . In the condenser that I use, with the loss angle mentioned, the lead angle was cut down to  $88^\circ$ , which is much better than can 20 be obtained in condensers where the dielectric is a solid or a liquid.

My improved insulator may be used

(1) As an insulating material for all kinds of cables applied either in the form of a band 25 or with an intermediate layer of paper, wood, fabric directly on the conductor,

(2) As insulation for high potential conductors, and as a protection against corona and other silent discharge,

(3) As insulating material for all kinds of 30 electric machines, as motors, dynamos, magnetos, and transformers,

(4) As a dielectric material for all kinds of condensers, either for high voltages or high 35 frequency,

(5) As a means to enable a large amount of energy to be accumulated in high powered condensers,

(6) As a means for obtaining great mechanical forces in a condenser with movable 40 plates.

As was stated, I obtained a polarized layer on an ordinary insulator, this polarized layer taking practically the entire potential drop 45 across it. An examination of this polarized layer showed that it was extremely poor in free ions. Furthermore, the thickness of this layer is such that the few free ions which are accelerated can only collide a very small 50 number of times and thus only a few ions are created. This means that only an infinitesimal current passes. Hence, an almost perfect insulating medium is thus created.

One method of creating such a layer is to 55 heat the insulator to a high temperature, though not high enough to permanently damage it, and at the same time pass a direct current of electricity through it. It has been found that when a direct potential is applied 60 to the opposite sides of an insulator by means of electrodes of appreciable area, there is initially a fairly large surge of current which is the so-called charging current. The value of current then drops down to a fairly low 65 value which continues to pass for a consider-

able length of time. It has been found, however, that this residual current decreases more and more until finally a very low value is reached. This action has been found to exist in insulators entirely free of any extraneous 70

current carriers, such as moisture or metallic particles. After a current has passed through it for some time under these conditions, the amount of current grows smaller and smaller, finally dropping to a very low 75

value. When this stage is reached, the current is stopped and the substance is allowed to cool. This method results in the production of a polarized layer. As stated above, 80

this polarized layer is extremely poor in free ions. Thus it will be noted that this process consists essentially in the removal of these 85

free ions from the surface layer. Inasmuch as the current which passes must result in the removal of the free ions, it is obvious that it 85

must be these free ions which conduct the current through the layer, and therefore the removal of these ions is what produces the decrease in the conductivity of said layer after 90

the current has been passing for a considerable length of time. It should be noted at this point that the potential applied must be in one direction in order that the ions have an opportunity to gradually progress to the surface of the insulator where they may escape 95

into the external circuit. In order to accomplish the removal of these ions, it is further obvious that the layer must be free of extraneous matter which would conduct the current, and therefore prevent this current from removing the free ions. Such extraneous matter 100

may be, for example, moisture or metallic particles and the like. I have treated pieces of glass, mica, colophony, thin layers of oil, benzol, linseed oil varnish, calcite, mother of 105

pearl, colloidal carbonic salts, aluminium oxides, phosphates and cements, etc. In all these cases, a polarized layer was formed and it was observed that with the thickness of this 110

layer within the limits mentioned above, the breakdown potential was practically independent of the thickness of the insulator. The polarized layer, moreover, will persist even when the substance has cooled.

Another method of producing such a layer 115 is by the action of air oxidizing the surface of the dielectric to be treated. Thus linseed oil is polymerized and purified at about  $250^\circ$  C. and then provided with a cobalt or manganese siccative.

This product is then superficially oxidized at about  $200^\circ$  C. In such a case, there appears to form a superficial layer of oxidized substance, which is permanent, and which has the property of being polarized 120

without the necessity of passing a current of electricity through it. In all such cases, thin layers in the neighborhood of .001 mm. were obtained—it is the polarized layer in all such 125

cases that is of this dimension, and not necessarily the entire insulating medium—which 130

successfully withstood a potential gradient of  $10^8$  volts per cm.

I claim:

- 5 1. An insulating body having its insulating strength concentrated in one or more thin layers of a thickness of the order of about five microns or less.
- 10 2. An insulating body comprising a plurality of layers, each of said layers comprising an insulating body having a thin layer of increased dielectric strength thereon, said thin layer being of a thickness of the order of between 1 and 5 microns.
- 15 3. The method of making an insulator resistant to high potential which consists in preparing a layer of material of very low conductivity, said conductivity depending practically solely on the presence of free ions in said layer, heating said layer, and causing a
- 20 20 current of electricity to go through it in one direction until the free ions are removed from a thin layer on the surface of said first-named layer, said removal being observed by the decrease of said current to a value considerably
- 25 25 less than its initial value.

In witness whereof I affix my signature.

ABRAHAM JOFFÉ.

30

35

40

45

50

55

60

65